



US005853903A

# United States Patent [19]

Hosoya et al.

[11] Patent Number: 5,853,903

[45] Date of Patent: Dec. 29, 1998

[54] STEEL SHEET FOR EXCELLENT PANEL APPEARANCE AND DENT RESISTANCE AFTER PANEL-FORMING

[75] Inventors: **Yoshihiro Hosoya; Fusato Kitano**, both of Fukuyama, Japan; **Yasunobu Nagataki**, Evanston, Ill.

[73] Assignee: **NKK Corporation**, Tokyo, Japan

[21] Appl. No.: **847,896**

[22] Filed: **Apr. 28, 1997**

[30] Foreign Application Priority Data

May 7, 1996 [JP] Japan ..... 8-137651

[51] Int. Cl.<sup>6</sup> ..... **B32B 15/01**

[52] U.S. Cl. ..... **428/669**; 148/320; 420/120; 420/121; 420/126; 420/127; 420/128

[58] Field of Search ..... 148/320; 420/120, 420/121, 126, 127, 128; 428/669

[56] References Cited

U.S. PATENT DOCUMENTS

4,496,400 1/1985 Irie et al. ..... 420/127  
4,750,952 6/1988 Sata et al. ..... 148/320  
5,133,815 7/1992 Hashimoto et al. ..... 148/319  
5,656,102 8/1997 Taylor et al. ..... 148/320  
5,690,755 11/1997 Yoshinaga et al. ..... 148/533

FOREIGN PATENT DOCUMENTS

0 572 666 A1 12/1993 European Pat. Off. .  
57-70258 4/1982 Japan .

61-276931 12/1986 Japan .  
3-277741 12/1991 Japan .  
4-2729 1/1992 Japan .  
4-173925 6/1992 Japan .  
7-278654 10/1995 Japan .

OTHER PUBLICATIONS

Patent Abstracts of Japan, vol. 096, No. 002, 29, Feb, 1996 of JP 07 278654 (Nippon Steel Corp), 24, Oct. 1995.

Patent Abstracts of Japan, vol. 016, No. 479 (C-0992), 6, Oct. 1992 of JP 04 173925 (Nissin Steel Co., LTD.) 22, Jun. 1992.

Database WPI, Section Ch, Week 9207, Derwent Publications Ltd., London, GB; Class M24, AN 92-054234 of JP 04 002 729 (Sumitomo Metal Ind. LTD.), 7, Jan. 1992.

Primary Examiner—John Sheehan

Attorney, Agent, or Firm—Frishauf, Holtz, Goodman, Langer & Chick, P.C.

[57]

ABSTRACT

A cold-rolled steel sheet or a zinc or zinc alloy layer coated steel sheet containing 0.0010 to 0.01 wt % of C and having a steel composition containing one or two kinds of 0.005 to 0.08 wt % of Nb and 0.01 to 0.07 wt % of Ti in the ranges given by  $\{(12/93)Nb+(12/48)Ti^*\} \geq 0.0005$ ,  $0 \leq C - \{(12/93)Nb+(12/48)Ti^*\} \leq 0.0015$ , and  $Ti^* = Ti - \{(48/32)S+(48/14)N\}$ , in which a bake hardenability BH f the steel sheet at 170° C.×20 min after 2% tensile prestrain is 10 to 35 MPa and the BH (MPa) and a yield strength YP (MPa) of the steel sheet satisfy the ranges given by  $BH \geq \exp(-0.115 \cdot YP + 23.0)$  and  $0.67 \cdot BH + 160 \leq YP \leq -0.8 \cdot BH + 280$ .

11 Claims, 8 Drawing Sheets



**FIG.1**

**FIG.2**

**FIG.3**

FIG.4



**FIG.5**

FIG.6



WORK-HARDENING EXPONENT (0.5~2% STRAIN):n

|   | STRAIN RATE                   |                               | REMARK            |
|---|-------------------------------|-------------------------------|-------------------|
|   | $3 \times 10^{-3}/\text{sec}$ | $3 \times 10^{-1}/\text{sec}$ |                   |
| ○ | $n \geq 0.25$                 | $n \geq 0.25$                 | PRESENT INVENTION |
| ◐ | $0.20 \leq n < 0.25$          |                               |                   |
| ◑ | $n < 0.20$                    |                               |                   |
| ● | $0.20 \leq n < 0.25$          | $n < 0.25$                    | COMPARISON        |
| ○ | $n < 0.20$                    |                               |                   |

\*  $\Delta W_{ca} > 0.2 \mu\text{m}$

FIG.7



FIG.8



| $\Delta W_{ca}$<br>( $\mu\text{m}$ ) | PLAIN-STRAIN |            |          |
|--------------------------------------|--------------|------------|----------|
|                                      | NONE         | PERMISSIVE | INFERIOR |
| 0                                    | ○            | ○          | ○        |
| $\leq 0.2$                           | ○            | ○          | ○        |
| $> 0.2$                              | ○            | ○          | ○        |

# STEEL SHEET FOR EXCELLENT PANEL APPEARANCE AND DENT RESISTANCE AFTER PANEL-FORMING

## BACKGROUND OF THE INVENTION

### 1. Field of the Invention

The present invention relates to a steel sheet used for outer panels of automobiles and the like, and more particularly, relates to a cold-rolled steel sheet, and a cold-rolled steel sheet coated with a zinc or zinc alloy layer having excellent formability and nonageing properties, and further, producing no surface defects at press-forming, and exhibiting excellent dent resistance after baking.

### 2. Description of the Related Art

As a matter of course, cold-rolled steel sheets used for outer panels of automobiles and the like are required to have excellent characteristics such as formability, shape fixability and surface uniformity(plane strain); and in addition, such characteristics are also required that automobile bodies with the steel sheets are not readily dented by a local external stress. Concerning the former characteristics, numerous techniques have been disclosed, according to which, parameters conventionally used for evaluating formability of steel sheet such as elongation, r value, and n value are improved. Meanwhile, concerning the latter characteristics, increasing the yield point of steel sheet has been investigated simultaneously with decreasing sheet thickness for lightening the automobile body weight to achieve reduction in cost of automotive fuel, since the dent load of steel sheet increases with Young's modulus, (sheet thickness)<sup>2</sup> and yield strength. However, an increase in the yield strength of steel sheet increases the spring back at press-forming, and thereby surface nonuniformity is readily produced around door handles in addition to deterioration of shape fixability. Conventionally, it has been known that surface nonuniformity is readily produced when the yield strength of steel sheet exceeds 240 MPa under normal press-forming conditions.

So-called BH steel sheets (steel sheets having bake hardenability), which have such characteristics that the yield strength is low at press-forming and is raised by a strain ageing phenomenon after baking (generally heating at 170° C. for approximately 20 min.), have been developed to solve the above problems and numerous improved techniques concerning this type of steel sheet have been disclosed. These BH steel sheets are characterized by a phenomenon, in which the yield strength increases due to strain ageing after baking by leaving a small amount of C in solid solution in the steel. However, when utilizing such a strain ageing phenomenon, ageing deterioration (reappearance of yield point elongation) more readily occurs in steel sheets during storage at room temperature as compared with nonageing steel sheets, thereby surface defects due to stretcher strain readily occur at press-forming.

Therefore, steel sheets having a two-phase structure have been developed as yield point elongation does not readily reappear in such steel sheets at ageing, in which two-phase structure, a low temperature transformation phase such as martensite dispersed in ferrite, is formed by a continuous annealing process. Although this type of steel sheet has BH as high as approximately 100 MPa, it is made of low carbon steel containing approximately 0.02 to 0.06 wt % of C; therefore this type of steel sheet cannot satisfy the formability required for today's outer panels of automobiles, and in addition, it cannot achieve the desired microstructure since it cannot be subjected to quenching or tempering when

steel sheet is hot-dip galvanized. Furthermore, deterioration in stretch-flangeability and the like specific to the two-phase structure steel prevents this type of steel sheet from being used for outer panels.

Meanwhile, so-called ultra-low carbon BH steel sheets have been developed by employing ultra-low carbon steel, containing not more than 0.005 wt % of C, and adding carbide forming elements such as Nb and Ti to the steel in quantities of not more than the stoichiometric ratio with respect to the C content; and these ultra-low carbon BH steel sheets can exhibit the bake hardenability due to residual C in solid solution while maintaining excellent properties specific to ultra-low carbon steel, such as deep drawability, and have been now widely applied to outer panels of automobiles and the like because this type of steel sheet is applicable to zinc or zinc alloy layer coated steel sheets. However, from a practical viewpoint, the BH of this type of steel sheet is reduced to approximately not more than 60 MPa because the steel sheet does not contain a hard second phase which can prevent reappearance of yield point elongation.

Conventionally, numerous improved techniques (for example, Japanese Unexamined Patent Publication No. 57-70258) concerning ultra-low carbon BH steel sheets have been proposed as follows: techniques of continuous annealing at a temperature as high as near 900° C. for elevating the r value by grain growth and raising the BH by redissolving carbide (for example, Japanese Unexamined Patent Publication No. 61-276931); and steel sheet manufacturing techniques aimed at suppressing the reappearance of yield point elongation, similar to the above-mentioned two-phase structure steel, in which a steel sheet is heated to around the  $Ac_3$  temperature and then cooled so as to obtain a recrystallized ferrite phase and a high dislocation density ferrite phase transformed from austenite (for example, Japanese Unexamined Patent Publication No. 3-277741).

However, each of these techniques requires annealing at a high temperature of not less than 880° to 900° C., thus they are not only disadvantageous in energy cost and productivity, but also readily form surface defects at press-forming due to coarse grain grown at high temperature annealing. In addition, since the high temperature annealing inevitably reduces the steel sheet's strength, the yield strength of the steel sheet after press-forming is not always high even when the BH is high, therefore a high BH alone does not always contribute to improvement in dent resistance.

## SUMMARY OF THE INVENTION

The object of the present invention is to provide a ultra-low carbon BH steel sheet which has substantially nonageing properties at room temperature, excellent formability, and excellent panel appearance after panel-forming, in addition to excellent dent resistance after baking.

The present invention is achieved by the following cold-rolled steel sheets:

A cold-rolled steel sheet 1, comprising a steel composition containing 0.0010 to 0.01 wt % of C, 0 to 0.2 wt % of Si, 0.1 to 1.5 wt % of Mn, 0 to 0.05 wt % of P, 0 to 0.02 wt % of S, 0.03 to 0.10 wt % of sol. Al, and 0 to 0.0040 wt % of N, and further containing one or two kinds of 0.005 to 0.08 wt % of Nb and 0.01 to 0.07 wt % of Ti in the ranges given by the following formulae (1) and (2):

$$\{(12/93)Nb + (12/48)Ti^*\} \geq 0.0005 \quad (1)$$

$$0 \leq C - \{(12/93)Nb + (12/48)Ti^*\} \leq 0.0015 \quad (2)$$

## 3

wherein  $Ti^* = Ti - \{(48/32)S + (48/14)N\}$

said cold-rolled steel sheet having a bake hardenability BH of 10 to 35 MPa obtained by 2% tensile prestrain and 170° C.×20 min heat treatment;

said bake hardenability BH (MPa) and a yield strength YP (MPa) of said steel sheet satisfying the following formulae (3a) and (4a)

$$BH \geq \exp(-0.115 \cdot YP + 23.0) \quad (3a)$$

$$0.67 \cdot BH + 160 \leq YP \leq -0.8 \cdot BH + 280 \quad (4a)$$

A cold-rolled steel sheet 2, comprising a steel composition containing 0.0010 to 0.01 wt % of C, 0 to 0.2 wt % of Si, 0.1 to 1.5 wt % of Mn, 0 to 0.05 wt % of P, 0 to 0.02 wt % of S, 0.03 to 0.10 wt % of sol. Al, and 0 to 0.0040 wt % of N, and further containing one or two kinds of 0.005 to 0.08 wt % of Nb and 0.01 to 0.07 wt % of Ti in the ranges given by the following formulae (1) and (2):

$$\{(12/93)Nb + (12/48)Ti^*\} \geq 0.0005 \quad (1)$$

$$0 \leq C - \{(12/93)Nb + (12/48)Ti^*\} \leq 0.0015 \quad (2)$$

wherein  $Ti^* = Ti - \{(48/32)S + (48/14)N\}$

said cold-rolled steel sheet having a bake hardenability BH of 10 to 30 MPa obtained by 2% tensile prestrain and 170° C.×20 min heat treatment;

said bake hardenability BH (MPa) and a yield strength YP (MPa) of said steel sheet satisfying the following formulae (3b) and (4b)

$$BH \geq \exp(-0.115 \cdot YP + 25.3) \quad (3b)$$

$$0.67 \cdot BH + 177 \leq YP \leq -0.8 \cdot BH + 260 \quad (4b)$$

A cold-rolled steel sheet 3, comprising a steel composition containing 0.0010 to 0.0025 wt % of C, 0 to 0.2 wt % of Si, 0.1 to 1.5 wt % of Mn, 0 to 0.05 wt % of P, 0 to 0.02 wt % of S, 0.03 to 0.10 wt % of sol. Al, and 0 to 0.0040 wt % of N, and further containing one or two kinds of 0.005 to 0.020 wt % of Nb and 0.01 to 0.05 wt % of Ti in the ranges given by the following formulae (1) and (2):

$$\{(12/93)Nb + (12/48)Ti^*\} \geq 0.0005 \quad (1)$$

$$0 \leq C - \{(12/93)Nb + (12/48)Ti^*\} \leq 0.0015 \quad (2)$$

wherein  $Ti^* = Ti - \{(48/32)S + (48/14)N\}$

said cold-rolled steel sheet having a bake hardenability BH of 10 to 35 MPa obtained by 2% tensile prestrain and 170° C.×20 min heat treatment;

said bake hardenability BH (MPa) and a yield strength YP (MPa) of said steel sheet satisfying the following formulae (3a) and (4a)

$$BH \geq \exp(-0.115 \cdot YP + 23.0) \quad (3a)$$

$$0.67 \cdot BH + 160 \leq YP \leq -0.8 \cdot BH + 280 \quad (4a)$$

A cold-rolled steel sheet 4, comprising a steel composition containing 0.0010 to 0.0025 wt % of C, 0 to 0.2 wt % of Si, 0.1 to 1.5 wt % of Mn, 0 to 0.05 wt % of P, 0 to 0.02 wt % of S, 0.03 to 0.10 wt % of sol. Al, and 0 to 0.0040 wt % of N, and further containing one or two kinds of 0.005 to 0.020 wt % of Nb and 0.01 to 0.05 wt % of Ti in the ranges given by the following formulae (1) and (2):

$$\{(12/93)Nb + (12/48)Ti^*\} \geq 0.0005 \quad (1)$$

$$0 \leq C - \{(12/93)Nb + (12/48)Ti^*\} \leq 0.0015 \quad (2)$$

## 4

wherein  $Ti^* = Ti - \{(48/32)S + (48/14)N\}$

said cold-rolled steel sheet having a bake hardenability BH of 10 to 30 MPa obtained by 2% tensile prestrain and 170° C.×20 min heat treatment;

said bake hardenability BH (MPa) and a yield strength YP (MPa) of said steel sheet satisfying the following formulae (3b) and (4b)

$$BH \geq \exp(-0.115 \cdot YP + 25.3) \quad (3b)$$

$$0.67 \cdot BH + 177 \leq YP \leq -0.8 \cdot BH + 260 \quad (4b)$$

It is also possible to achieve the present invention by a cold-rolled steel sheet 1, wherein said steel composition contains 0.0002 to 0.0015 wt % of B or wherein said cold-rolled steel sheet is coated with a zinc or zinc alloy layer.

## BRIEF DESCRIPTION OF THE DRAWINGS

FIG. 1 is a graph which shows the effects of the 2% BH of an ultra-low carbon cold-rolled steel sheet and a low carbon cold-rolled steel sheet on stretchability ( $LDH_0$ ).

FIG. 2 is a graph which shows the effects of the 2% BH of an ultra-low carbon cold-rolled steel sheet and a low carbon cold-rolled steel sheet on the limiting drawing ratio (LDR).

FIG. 3 is a schematic drawing which illustrates a forming method and the shape of a model-panel used for investigation.

FIG. 4 is a graph which shows the effects of the 2% BH of an ultra-low carbon cold-rolled steel sheet and a low carbon cold-rolled steel sheet, each formed into a model panel as shown in FIG. 3 after artificial ageing at 38° C.×6 months, on the changes ( $\Delta Wca$ ) in waviness heights (Wca) measured before and after panel-forming.

FIG. 5 is a graph which shows the effects of the 2% BH of an ultra-low carbon cold-rolled steel sheet and a low carbon cold-rolled steel sheet on the dent resistance (dent load) of panels.

FIG. 6 is a graph shows the effects of C content on the work-hardening exponent n and  $\Delta Wca$  of the steel sheet evaluated at two kinds of strain rates.

FIG. 7 is a graph shows the effects of YP and the 2% BH of an ultra-low carbon cold-rolled steel sheet on the dent resistance (dent load) of a panel which has been formed into a model-panel as shown in FIG. 3, followed by baking at 170° C.×20 min.

FIG. 8 is a graph which shows the effects of YP and the 2% BH of an ultra-low carbon cold-rolled steel sheet on the changes ( $\Delta Wca$ ) in waviness heights (Wca) measured before and after forming the steel sheet into a model-panel as shown in FIG. 3, followed by baking at 170° C.×20 min and on the surface nonuniformity around a handle when the steel sheet is formed into a model-panel having a bulged part on a flat portion of the panel corresponding to a door handle seat.

## DESCRIPTION OF THE PREFERRED EMBODIMENTS

To solve the problems of conventional ultra-low carbon BH steel sheets, the inventors of the present invention have investigated factors controlling dent resistance in detail, and as a result, have had the following findings. In other words, although the bake hardenability was advantageous to some extent in elevating the yield strength of steel sheets, the

contribution of the BH to dent resistance was relatively small when the BH of steel sheets was not more than 50 MPa, and on the contrary, the following phenomena were found to have more adverse effects on not only dent resistance but also panel appearance: reduction in the  $r$  value or the  $n$  value inevitably caused by leaving more than C in solid solution disturbed the flow of steel sheets into the panel face from the flange portion at panel-forming and impeded work-hardening of the steel sheets by uniform strain propagation over the panel face. In other words, contrary to conventional knowledge "to increase the bake hardenability is the best way to improve dent resistance of outer panel of automobiles", it has been apparent that an increase in the bake hardenability does not always lead to improvement in dent resistance. Meanwhile, it was also found that when the 10 bake hardenability was not less than 35 MPa, yield point elongation reappeared during long term storage after temper rolling, resulting in surface defects at panel-forming which are fatal for outer panels, in addition to deterioration of elongation.

In the following, a process to achieve the present invention and characteristics of the present invention will be explained.

First, the effects of the 2% BH on formability of steel sheets and surface defects after panel-forming were studied. In this study, 0.7 mm thick ultra-low carbon cold-rolled steel sheets (0.0015 to 0.0042 wt % of C, 0.01 to 0.02 wt % of Si, 0.5 to 0.6 wt % of Mn, 0.03 to 0.04 wt % of P, 0.008 to 0.011 wt % of S, 0.040 to 0.045 wt % of sol. Al, 0.0020 to 0.0024 wt % of N, and 0.005 to 0.012 wt % of Nb) and 0.7 mm thick low carbon cold-rolled steel sheets (0.028 to 0.038 wt % of C, 0.01 wt % of Si, 0.15 to 0.16 wt % of Mn, 0.02 to 0.03 wt % of P, 0.005 to 0.010 wt % of S, 0.035 to 0.042 wt % of sol. Al, and 0.0025 to 0.0030 wt % of N), with different 15 20 25 30 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 498 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 547

a viewpoint of dent resistance of the panel immediately after panel-forming, the assemblability and the like, it is preferable to provide a 2% BH of not less than 10 MPa to steel sheets applied to outer panels of automobiles. Thus, the lower limit of 2% BH for ultra-low carbon BH steel sheets is set to 10 MPa in the present invention.

An investigation was carried out on work-hardening behavior at two kinds of strain rates in a strain region of not more than 5%, which behavior is regarded to be an important characteristic contributing to dent resistance. FIG. 6 shows the results of a study on the effects of C content on the work-hardening exponent  $n$  and the  $\Delta W_{ca}$  at panel-forming in a small strain region of 0.5 to 2% at a static strain rate of  $3 \times 10^{-3}/s$  and at a dynamic strain rate of  $3 \times 10^{-1}/s$  similar to the actual press condition, using 0.7 mm thick ultra-low carbon cold-rolled steel sheets containing 0.0005 to 0.011 wt % of C, 0.01 to 0.02 wt % of Si, 0.5 to 0.6 wt % of Mn, 0.03 to 0.04 wt % of P, 0.008 to 0.011 wt % of S, 0.040 to 0.045 wt % of sol. Al, 0.0020 to 0.0024 wt % of N, 0 to 0.08 wt % of Nb, and 0 to 0.07 wt % of Ti.

From FIG. 6, high  $n$  values are obtained at a dynamic strain rate of  $3 \times 10^{-1}/s$  under such conditions that the total C is not more than 100 ppm,  $\{(12/93)Nb + (12/48)Ti^*\}$ , which is a parameter indicating precipitation amount of carbon (which carbon precipitates as NbC or TiC in a ferrite phase) in an equilibrium condition, is not less than 5 ppm, and  $C - \{(12/93)Nb + (12/48)Ti^*\}$ , which is a parameter indicating C in solid solution in an equilibrium condition, is not less than 15 ppm, wherein  $Ti^* = Ti - \{(48/32)S + (48/14)N\}$ . The high  $n$  values are obtained even at a static strain rate of  $3 \times 10^{-3}/s$  when the total C is not more than 25 ppm. In the same way as in FIG. 4, the relation  $\Delta W_{ca} \leq 0.2 \mu m$  is obtained when  $C - \{(12/93)Nb + (12/48)Ti^*\}$  is not more than 15 ppm. Furthermore, when the above parameters are not less than 0 ppm, BH of not less than 10 MPa can be ensured. Therefore, in ultra-low carbon steel sheets of which steel composition contains one or two kinds of Nb and Ti, it is necessary that Nb and Ti satisfy  $\{(12/93)Nb + (12/48)Ti^*\} \geq 0.0005$  and  $0 \leq C - \{(12/93)Nb + (12/48)Ti^*\} \leq 0.0015$ . Therefore, in the present invention, the contents of Nb and Ti in the steel composition are set to the ranges given by the following formulae (1) and (2):

$$\{(12/93)Nb + (12/48)Ti^*\} \geq 0.0005 \quad (1)$$

$$0 \leq C - \{(12/93)Nb + (12/48)Ti^*\} \leq 0.0015 \quad (2)$$

wherein  $Ti^* = Ti - \{(48/32)S + (48/14)N\}$ .

The following investigation was preformed on the most important factors of the present invention, i. e., the yield strength before panel-forming and the 2% BH from a viewpoint of ensuring dent resistance after panel-forming. Ultra-low carbon cold-rolled steel sheets (0.0005 to 0.012 wt % of C, 0.01 to 0.02 wt % of Si, 0.5 to 0.6 wt % of Mn, 0.03 to 0.04 wt % of P, 0.008 to 0.011 wt % of S, 0.040 to 0.045 wt % of sol. Al, 0.0020 to 0.0024 wt % of N, and 0.0020 to 0.08 wt % of Nb) having various yield strength values and 2% BH were panel-formed into a model-panel as shown in FIG. 3, subjected to heat treatment corresponding to a baking process, followed by evaluation of  $\Delta W_{ca}$  in the center portion of the panel face. In addition, a load (dent load) causing a 0.1 mm permanent dent by pushing a 50 mmR ball-point punch on the center of a flat portion of the panel was measured. Moreover, the same steel sheets were panel-formed into panels having the same shape as that shown in FIG. 3 with a bulge-formed part on its flat portion corresponding to a door handle seat so as to investigate plane strain around the handle. FIGS. 7 and 8 show the results.

FIGS. 7 and 8 indicate that the dent load of a panel is raised by increasing the initial yield strength  $Y_P$  and the 2% BH. With regard to the effect of  $Y_P$ , the dent load rapidly decreases in a region where  $Y_P$  is not more than 170 MPa, thus it is necessary to set the 2% BH to not less than 40 MPa for compensation. Meanwhile, concerning the effect of the 2% BH, the dent load rapidly decreases in a region in which the 2% BH is not more than 10 MPa, and a dent load of not less than 150N cannot be achieved in a substantial nonaging steel sheet having a 2% BH of less than 1 MPa. In a region in which  $Y_P$  is not more than 200 MPa, critical conditions exist between  $Y_P$  and the 2% BH for dent load, and it is necessary to have a 2% BH of  $BH \geq \exp(-0.115 \cdot Y_P + 23.0)$  for achieving dent resistance having a dent load of not less than 150N and to have a 2% BH of  $BH \geq \exp(-0.115 \cdot Y_P + 25.3)$  for achieving dent resistance having a dent load of not less than 170N, respectively. Therefore, according to the present invention, the 2% BH (MPa) and the yield strength  $Y_P$  (MPa) of a steel sheet are regulated to satisfy the following formula (3a), and preferably, the following formula (3b) from a viewpoint of ensuring excellent dent resistance:

$$BH \geq \exp(-0.115 \cdot Y_P + 23.0) \quad (3a)$$

$$BH \geq \exp(-0.115 \cdot Y_P + 25.3) \quad (3b)$$

In addition, it is necessary to set the 2% BH and  $Y_P$  to appropriate values from a viewpoint of excellent panel appearance required for outer panels. Surface defects of a panel become remarkable with a decrease in  $Y_P$  and an increase in the 2% BH, as is shown in FIG. 8. Meanwhile, surface nonuniformity around handle becomes remarkable with an increase in  $Y_P$  and a decrease in the 2% BH. From the above results, concerning the conditions for the 2% BH and  $Y_P$ , a 2% BH of not more than 35 MPa and  $0.67 \cdot BH + 160 \leq Y_P \leq -0.8 \cdot BH + 280$  are required so as not to have practical problems in surface defects of the panel face or surface nonuniformity around the handle; and a 2% BH of not more than 30 MPa and  $0.67 \cdot BH + 177 \leq Y_P \leq -0.8 \cdot BH + 260$  are required so as not to have any surface defects of the panel face nor surface nonuniformity around the handle. Therefore, in the present invention, the 2% BH (MPa) and the yield strength  $Y_P$  (MPa) of a steel sheet are regulated to satisfy the following formula (4a), and preferably, the following formula (4b):

$$0.67 \cdot BH + 160 \leq Y_P \leq -0.8 \cdot BH + 280 \quad (4a)$$

$$0.67 \cdot BH + 177 \leq Y_P \leq -0.8 \cdot BH + 260 \quad (4b)$$

50 The reasons for limiting the composition of steel sheets of the present invention will be explained.

C: As is above-mentioned, in the present invention, it is necessary to set the amounts of fine precipitates such as NbC and TiC precipitating in steel to not less than 5 ppm expressed as the corresponding C amount (equilibrium condition), in addition to ensuring C in solid solution for obtaining a 2% BH of not less than 10 MPa. When the total C in a steel sheet is less than 0.0010 wt %, the required 2% BH cannot be obtained, and meanwhile, if the C exceeds 0.01 wt %, the work-hardening exponent  $n$  decreases. Therefore the total C is set from 0.0010 to 0.01 wt %, and preferably not more than 0.0025 wt % for the high  $n$  value as above-mentioned.

Si: When an exceedingly large amount of Si is added, chemical conversion treatment properties deteriorate in the case of cold-rolled steel sheets, and adhesion of layer deteriorates in the case of zincor zinc alloy layer coated steel

sheets; therefore the amount of Si is set to not more than 0.2 wt % (including 0 wt %).

Mn: Mn is an indispensable element in steel because it serves to prevent hot shortness of a slab by precipitating S as MnS in the steel. In addition, Mn is an element which can solid solution strengthen the steel without deteriorating adhesion of zinc plating layer. However, addition of an exceedingly large amount of Mn is not preferable because it results in a deteriorated r value and an excessively increased yield strength. Therefore, the lower limit of Mn is 0.1 wt % which value is a minimum requirement for precipitating and anchoring S, and the upper limit is 1.5 wt % which value is a limit for avoiding remarkably deteriorated r values and for not exceeding the yield strength of 240 MPa.

P: Since P deteriorates the alloying properties at hot-dip galvanizing and also causes a surface defect on the panel face due to microsegregation of P, the amount of P is preferably as small as possible and set to not more than 0.05 wt % (including 0 wt %).

S: S is included as MnS in steel, and if a steel sheet contains Ti, S precipitates as  $Ti_4C_2S_2$  in the steel; since an excess amount of S deteriorates stretch-flangeability and the like, the amount of S is set to not more than 0.02 wt % (including 0 wt %), in which range no problems occur in practical formability or surface treatability.

sol. Al: Sol. Al has a function of precipitating N as AlN in steel and reducing harmful effects due to N in solid solution, which harmful effects decrease the ductility of steel sheets by a dynamic strain ageing, similarly to C in solid solution. When the amount of sol. Al is less than 0.03 wt %, the above effects cannot be achieved, and meanwhile, addition of more than 0.10 wt % of sol. Al does not lead to further effects corresponding to the added amount; therefore the amount of sol. Al is set to 0.03 to 0.10 wt %.

N: Although N is rendered harmless by precipitating as AlN and also precipitating as BN when B is added, the amount of N is preferably as small as possible from a viewpoint of steelmaking techniques, therefore N is set to not more than 0.0040 wt % (including 0 wt %).

Nb and Ti: One or two kinds of 0.005 to 0.08 wt % of Nb and 0.01 to 0.07 wt % of Ti are added to a steel sheet of the present invention as essential elements. These elements are added to steel for controlling the amounts of fine precipitates in the steel such as NbC, TiC, etc. to not less than 5 ppm, which value is expressed by the corresponding C amount in steel (under equilibrium conditions), so as to increase the work-hardening exponent n in an initial deformation stage, and also for anchoring the excess C as NbC or TiC so as to control the amount of residual C in solid solution to not more than 15 ppm. When the added amounts of Nb and Ti are below 0.005 wt % for Nb and 0.01 wt % for Ti respectively, the above-mentioned control of precipitating C cannot be performed appropriately, and meanwhile, if the added amounts of Nb and Ti exceed the 0.08 wt % for Nb and 0.07 wt % for Ti respectively, it becomes difficult to ensure the C in solid solution required for achieving the desired BH properties. These upper limits are more preferably set to 0.020 wt % for Nb and 0.05 wt % for Ti respectively.

B: Although the above-mentioned composition limitations are sufficient for achieving the present invention, addition of 0.0002 to 0.0015 wt % of B is advantageous in further stabilizing the surface quality and dent resistance. The  $Ar_3$  transforming temperature falls due to the addition of B and results in a uniform fine structure over the full length and width of ultra-low carbon hot-rolled steel sheet, and consequently, the surface quality after cold-rolling and annealing is improved; and a small amount of B segregated

in ferrite grain boundaries during annealing prevents the C in solid solution from precipitating in grain boundaries during cooling, thus a relatively stable amount of C in solid solution can be left in the steel without high temperature annealing. When the added amount of B is less than 0.0002 wt %, the above-mentioned effects cannot be sufficiently obtained; and meanwhile, formability such as deep drawability deteriorates when the added amount exceeds 0.0015 wt %. Therefore, in the case of adding B, the added amount thereof is set to 0.0002 to 0.0015 wt %.

Balance: Although the balance is substantially composed of Fe, other elements may be added within the limit of not deteriorating the above-mentioned effects of the present invention.

Although steel sheets of the present invention can be used as a cold-rolled sheet, they can be also used as a zinc or a zinc alloy layer coated steel sheet by zinc electroplating or hot-dip galvanizing the cold-rolled steel sheet, and also in this case, the desired surface quality and dent resistance can be obtained after press-forming.

Pure zinc plating, alloyed zinc plating, zinc Ni alloy plating, etc. are employed as the zinc or zinc alloy layer coating, and similar properties can be achieved in steel sheets treated by organic coating after zinc plating.

A example method for manufacturing steel sheets of the present invention will be explained.

A steel sheet of the present invention is manufactured through a series of manufacturing processes including hot-rolling, pickling, cold rolling, annealing, and treated with zinc plating if required. For manufacturing a steel sheet of the present invention, it is preferred that the finishing temperature of the hot-rolling be set to not less than the  $Ar_3$  temperature so as to ensure excellent surface quality and uniform properties required for outer panels. In addition, although either of a method of hot-rolling after slab-heating or a method of hot-rolling without slab-heating can be employed for the hot-rolling process, it is preferred that not only the primary scales but also the second scales producing at hot rolling be sufficiently removed for the outer panels. In addition, the preferred coiling temperature after hot-rolling is not more than 680° C., and more preferably, not more than 660° C., from a viewpoints of scale-removal at pickling and stability of the product properties. Furthermore, the preferred lower limit of the coiling temperature is 600° C. for continuous annealing and 540° C. for box annealing so as to avoid adverse effects on a recrystallization texture formation by growing carbide to some extent.

For cold-rolling the hot-rolled steel sheet after scale-removal, it is preferred to set the cold-rolling reduction rate to not less than 70%, and more preferably not less than 75% to achieve the deep-drawability required for outer panels. In addition, when continuous annealing is employed for annealing the cold-rolled steel sheet, the preferred annealing temperature is 780° to 880° C. and more preferably, 780° to 860° C. This is because annealing at temperature of not less than 780° C. is necessary for developing the desired texture for the deep-drawability after recrystallization, and meanwhile, at annealing temperature of more than 860° C.,  $Y_p$  decreases and also remarkable surface defects appear at panel-forming. On the other hand, when box annealing is employed for annealing, a uniform recrystallization structure can be obtained at annealing temperature of not less than 680° C. because of the long soaking time of box annealing, however, the preferred upper limit of the annealing temperature is 750° C. for suppressing grain coarsening.

The annealed cold-rolled steel sheet can be subjected to zinc or zinc alloy layer coating by zinc electroplating or hot-dip galvanizing.

## 11

## (EXAMPLE 1)

Steels of steel No. 1 to No. 30 each having a composition shown in Tables 1 and 2 were melted and continuously cast into 220 mm thick slabs. These slabs were heated to 1200° C. and then hot-rolled into 2.8 mm thick hot-rolled sheets at finishing temperature of 860° C. (steel No. 1) and 880° to 910° C. (steel Nos. 2 to 30), and at coiling temperature of 540° to 560° C. (for box annealing) and 600° to 640° C. (for continuous annealing and continuous annealing hot-dip galvanizing). These hot-rolled sheets were pickled, cold-rolled to 0.7 mm thickness, followed by one of the following annealing processes: continuous annealing (840° to 860° C.), box annealing (680° to 720° C.), and continuous annealing hot-dip galvanizing (850° to 860° C.). In continuous annealing hot-dip galvanizing, the hot-dip galvanizing was performed at 460° C. after annealing and then the resultant was immediately subjected to alloying treatment in an inline alloying furnace at 500° C. In addition, steel sheets after annealing or annealing hot-dip galvanizing were subjected to temper rolling at a rolling reduction of 1.2%.

The mechanical characteristics of the steel sheets were measured at a static strain rate of  $3 \times 10^{-3}/s$ . The work-hardening exponent  $n$  was also measured at a dynamic strain rate of  $3 \times 10^{-1}/s$  to evaluate the work-hardening behavior under actual press conditions. And these steel sheets were press-formed to evaluated: LDH<sub>0</sub> (limiting stretchability height) and LDR (limiting drawing ratio) by forming cy-

## 12

inders with a diameter of 50 mm; surface defects, plane strain, and dent resistance when formed into a panel as shown in FIG. 3; and further, dent resistance after baking. Tables 3 to 5 show the results thereof.

5

## (EXAMPLE 2)

Steels of steel No. 6, No. 6, No. 12, No. 21, No. 25, and No. 26, each having a composition shown in Tables 1 and 2 were melted and continuously cast into 220 mm thick slabs. These slabs were heated to 1200° C. and then hot-rolled to 2.8 mm thick at finishing temperature of 880° to 900° C. and coiling temperature of 640° to 720° C. These hot-rolled sheets were pickled, cold-rolled to 0.7 mm thickness, and subjected to continuous annealing at 840° to 920° C., followed by temper rolling at a rolling reduction of 1.2%.

These steel sheets were press-formed to evaluated: LDH<sub>0</sub> (limiting stretchability height) and LDR (limiting drawing ratio) by forming cylinders with a diameter of 50 mm; surface defects, plane strain, and dent resistance when formed into a panel as shown in FIG. 3; and further, dent resistance after baking. Tables 6 to 7 show the results thereof with characteristic values of steel sheets.

As is mentioned in the above, steel sheets of the present invention have substantial nonageing properties at room temperature, excellent formability, and excellent panel appearance after panel-forming, in addition to excellent dent resistance after baking. Tables 6 to 7 show the results thereof

| Steel | Composition(wt %) |        |      |      |       |       |       |        |       |    |        | X<br>(wt %) | Y<br>(wt %) |        |
|-------|-------------------|--------|------|------|-------|-------|-------|--------|-------|----|--------|-------------|-------------|--------|
|       | No.               | Type   | C    | Si   | Mn    | P     | S     | sol.Al | N     | Nb | Ti     | B           |             |        |
| 1     | C                 | 0.031  | 0.01 | 0.15 | 0.023 | 0.012 | 0.036 | 0.0022 | —     | —  | —      | —           | —           | —      |
| 2     | C                 | 0.0019 | 0.02 | 0.62 | 0.045 | 0.013 | 0.037 | 0.0019 | —     | —  | —      | —           | —           | —      |
| 3     | C                 | 0.0022 | 0.01 | 0.53 | 0.032 | 0.009 | 0.039 | 0.0022 | —     | —  | 0.0015 | —           | —           | —      |
| 4     | I                 | 0.0019 | 0.02 | 0.56 | 0.035 | 0.011 | 0.044 | 0.0021 | 0.006 | —  | —      | —           | 0.0007      | 0.001  |
| 5     | I                 | 0.0023 | 0.01 | 0.48 | 0.028 | 0.009 | 0.045 | 0.0018 | 0.011 | —  | —      | —           | 0.0013      | 0.001  |
| 6     | C                 | 0.0022 | 0.01 | 0.47 | 0.027 | 0.014 | 0.043 | 0.0018 | 0.021 | —  | —      | —           | 0.0026      | 0.000  |
| 7     | I                 | 0.0018 | 0.02 | 0.92 | 0.032 | 0.007 | 0.054 | 0.0016 | 0.009 | —  | —      | —           | 0.0011      | 0.001  |
| 8     | C                 | 0.0029 | 0.01 | 0.52 | 0.033 | 0.011 | 0.053 | 0.0015 | 0.011 | —  | —      | —           | 0.0013      | 0.002  |
| 9     | C                 | 0.0035 | 0.01 | 0.49 | 0.027 | 0.011 | 0.052 | 0.0023 | 0.015 | —  | —      | —           | 0.0018      | 0.002  |
| 10    | I                 | 0.0022 | 0.01 | 0.25 | 0.029 | 0.012 | 0.043 | 0.0025 | 0.009 | —  | —      | —           | 0.0011      | 0.001  |
| 11    | C                 | 0.0023 | 0.02 | 0.26 | 0.027 | 0.009 | 0.044 | 0.0025 | 0.022 | —  | —      | —           | 0.0027      | 0.000  |
| 12    | I                 | 0.0019 | 0.01 | 1.25 | 0.014 | 0.009 | 0.041 | 0.0024 | 0.015 | —  | —      | —           | 0.0018      | 0.000  |
| 13    | C                 | 0.0019 | 0.01 | 0.42 | 0.031 | 0.010 | 0.038 | 0.0026 | 0.022 | —  | —      | —           | 0.0027      | -0.001 |
| 14    | C                 | 0.0008 | 0.02 | 0.58 | 0.031 | 0.008 | 0.037 | 0.0022 | 0.011 | —  | —      | —           | 0.0013      | -0.001 |
| 15    | I                 | 0.0021 | 0.02 | 0.43 | 0.034 | 0.012 | 0.042 | 0.0021 | 0.011 | —  | 0.0008 | 0.0013      | 0.001       |        |
| 16    | C                 | 0.0029 | 0.01 | 0.41 | 0.035 | 0.015 | 0.045 | 0.0019 | 0.011 | —  | 0.0009 | 0.0013      | 0.002       |        |
| 17    | C                 | 0.0038 | 0.01 | 0.42 | 0.036 | 0.014 | 0.048 | 0.0020 | 0.018 | —  | 0.0007 | 0.0022      | 0.002       |        |

I: Invention, C: Comparison

X: (12/93)Nb + (12/48)Ti\*

Y: C-{(12/93)Nb + (12/48)Ti\*}

Ti: Ti-{(48/32)S + (48/14)N}

TABLE 2

| Steel | Composition(wt %) |        |      |      |       |       |       |        |       |       |    | X<br>(wt %) | Y<br>(wt %) |
|-------|-------------------|--------|------|------|-------|-------|-------|--------|-------|-------|----|-------------|-------------|
|       | No.               | Type   | C    | Si   | Mn    | P     | S     | sol.Al | N     | Nb    | Ti | B           |             |
| 18    | I                 | 0.0050 | 0.02 | 0.35 | 0.042 | 0.010 | 0.051 | 0.0022 | 0.029 | —     | —  | 0.0037      | 0.0013      |
| 19    | I                 | 0.0070 | 0.01 | 0.66 | 0.025 | 0.011 | 0.041 | 0.0019 | 0.046 | —     | —  | 0.0059      | 0.0011      |
| 20    | C                 | 0.0090 | 0.01 | 0.51 | 0.033 | 0.012 | 0.047 | 0.0020 | 0.054 | —     | —  | 0.0070      | 0.0020      |
| 21    | C                 | 0.0120 | 0.02 | 0.37 | 0.028 | 0.010 | 0.055 | 0.0023 | 0.08  | —     | —  | 0.0103      | 0.0017      |
| 22    | I                 | 0.0021 | 0.01 | 0.52 | 0.039 | 0.009 | 0.048 | 0.0018 | —     | 0.023 | —  | 0.0008      | 0.0013      |
| 23    | I                 | 0.0021 | 0.02 | 0.53 | 0.038 | 0.012 | 0.045 | 0.0028 | —     | 0.032 | —  | 0.0011      | 0.0010      |
| 24    | I                 | 0.0022 | 0.01 | 0.53 | 0.039 | 0.018 | 0.052 | 0.0039 | —     | 0.045 | —  | 0.0012      | 0.0010      |
| 25    | C                 | 0.0021 | 0.02 | 0.49 | 0.035 | 0.015 | 0.053 | 0.0025 | —     | 0.066 | —  | 0.0087      | -0.0066     |
| 26    | C                 | 0.0037 | 0.01 | 0.45 | 0.034 | 0.011 | 0.053 | 0.0024 | —     | 0.055 | —  | 0.0076      | -0.0039     |
| 27    | I                 | 0.0023 | 0.01 | 0.48 | 0.025 | 0.012 | 0.044 | 0.0022 | 0.009 | 0.025 | —  | 0.0010      | 0.0013      |

TABLE 2-continued

| Steel |      | Composition(wt %) |      |      |       |       |        |        |       |       | X      | Y      |         |
|-------|------|-------------------|------|------|-------|-------|--------|--------|-------|-------|--------|--------|---------|
| No.   | Type | C                 | Si   | Mn   | P     | S     | sol.Al | N      | Nb    | Ti    | B      | (wt %) | (wt %)  |
| 28    | C    | 0.0035            | 0.01 | 0.49 | 0.027 | 0.013 | 0.043  | 0.0024 | 0.012 | 0.038 | —      | 0.0040 | -0.0005 |
| 29    | C    | 0.0019            | 0.02 | 0.52 | 0.025 | 0.009 | 0.042  | 0.0018 | 0.023 | 0.024 | —      | 0.0039 | -0.0020 |
| 30    | I    | 0.0019            | 0.01 | 0.53 | 0.024 | 0.009 | 0.066  | 0.0017 | 0.014 | 0.018 | —      | 0.0014 | 0.0005  |
| 31    | I    | 0.0085            | 0.01 | 0.37 | 0.030 | 0.01  | 0.051  | 0.0018 | 0.04  | 0.03  | —      | 0.0074 | 0.0011  |
| 32    | I    | 0.0024            | 0.01 | 0.43 | 0.032 | 0.011 | 0.062  | 0.0026 | —     | 0.033 | 0.0009 | 0.0019 | 0.0005  |
| 33    | C    | 0.0029            | 0.01 | 0.42 | 0.033 | 0.012 | 0.054  | 0.0024 | —     | 0.052 | 0.0007 | 0.0064 | -0.0035 |
| 34    | I    | 0.0021            | 0.02 | 0.38 | 0.023 | 0.008 | 0.052  | 0.0019 | 0.009 | 0.018 | 0.0005 | 0.0010 | 0.0011  |
| 35    | C    | 0.0033            | 0.02 | 0.39 | 0.022 | 0.011 | 0.055  | 0.0016 | 0.011 | 0.022 | 0.0007 | 0.0014 | 0.0019  |

TABLE 3

| No. | Steel | Mechanical properties |           |             |             |                            |                            |              | Dent load  |                 |              |                   | after         |  |
|-----|-------|-----------------------|-----------|-------------|-------------|----------------------------|----------------------------|--------------|------------|-----------------|--------------|-------------------|---------------|--|
|     |       | No.                   | Annealing | YP<br>(MPa) | BH<br>(MPa) | Strain rate<br>:3 × 10-3/s | Strain rate<br>:3 × 10-1/s | LDH0<br>(mm) | LDR        | Formabilities   |              | Panel performance |               |  |
|     |       |                       |           |             |             |                            |                            |              |            | Plane<br>strain | ΔWca<br>(μm) | Dent load<br>(N)  | baking<br>(N) |  |
| 1   | 1     | CAL                   | 238       | 56          | 0.159       | 0.162                      | 26.8                       | 1.98         | Inferior   | 0               | 112          | 185               |               |  |
| 2   |       | BAF                   | 231       | 0           | 0.183       | 0.186                      | 28.3                       | 2.05         | None       | 0               | 101          | 172               |               |  |
| 3   |       | CGL                   | 242       | 63          | 0.145       | 0.153                      | 26.7                       | 1.96         | Inferior   | 0               | 113          | 184               |               |  |
| 4   | 2     | CAL                   | 182       | 31          | 0.194       | 0.196                      | 29.3                       | 2.01         | None       | 0.6             | 89           | 162               |               |  |
| 5   |       | BAF                   | 163       | 12          | 0.213       | 0.211                      | 30.5                       | 2.09         | None       | 0.8             | 65           | 141               |               |  |
| 6   |       | CGL                   | 185       | 34          | 0.175       | 0.177                      | 28.7                       | 1.99         | None       | 0.6             | 90           | 165               |               |  |
| 7   | 3     | CAL                   | 189       | 18          | 0.179       | 0.183                      | 29.8                       | 2.04         | None       | 0               | 93           | 159               |               |  |
| 8   | 4     | CAL                   | 208       | 25          | 0.262       | 0.266                      | 31.4                       | 2.14         | None       | 0               | 95           | 175               |               |  |
| 9   |       | CGL                   | 210       | 28          | 0.249       | 0.255                      | 31.2                       | 2.13         | None       | 0               | 96           | 176               |               |  |
| 10  | 5     | CAL                   | 217       | 22          | 0.275       | 0.273                      | 30.9                       | 2.13         | None       | 0               | 92           | 178               |               |  |
| 11  |       | BAF                   | 208       | 17          | 0.262       | 0.263                      | 30.1                       | 2.91         | None       | 0               | 88           | 172               |               |  |
| 12  |       | CGL                   | 218       | 26          | 0.256       | 0.261                      | 30.8                       | 2.13         | None       | 0               | 92           | 177               |               |  |
| 13  | 6     | CAL                   | 203       | 0           | 0.237       | 0.197                      | 31.1                       | 2.16         | None       | 0               | 58           | 145               |               |  |
| 14  |       | BAF                   | 198       | 0           | 0.223       | 0.216                      | 30.5                       | 2.15         | None       | 0               | 69           | 139               |               |  |
| 15  |       | CGL                   | 205       | 0           | 0.231       | 0.193                      | 31                         | 2.15         | None       | 0               | 57           | 143               |               |  |
| 16  | 7     | CAL                   | 235       | 16          | 0.269       | 0.271                      | 31.4                       | 2.15         | None       | 0               | 89           | 183               |               |  |
| 17  |       | CGL                   | 234       | 19          | 0.252       | 0.256                      | 31.2                       | 2.14         | None       | 0               | 92           | 184               |               |  |
| 18  | 8     | CAL                   | 238       | 37          | 0.227       | 0.252                      | 29.5                       | 2.08         | Permissive | 0.2             | 94           | 179               |               |  |
| 19  | 9     | CAL                   | 247       | 39          | 0.195       | 0.251                      | 29                         | 2.06         | Permissive | 0.2             | 96           | 181               |               |  |
| 20  | 10    | CAL                   | 196       | 28          | 0.267       | 0.265                      | 30.9                       | 2.15         | None       | 0               | 95           | 174               |               |  |
| 21  |       | CGL                   | 193       | 24          | 0.253       | 0.259                      | 30.8                       | 2.14         | None       | 0               | 95           | 175               |               |  |

CAL: Continuous annealing

BAF: Box annealing

CGL : Continuous annealing hot-dip galvanizing

TABLE 4

| No. | Steel | Mechanical properties |           |             |             |                            |                            |              | Dent load  |                 |              |                   | after         |  |
|-----|-------|-----------------------|-----------|-------------|-------------|----------------------------|----------------------------|--------------|------------|-----------------|--------------|-------------------|---------------|--|
|     |       | No.                   | Annealing | YP<br>(MPa) | BH<br>(MPa) | Strain rate<br>:3 × 10-3/s | Strain rate<br>:3 × 10-1/s | LDH0<br>(mm) | LDR        | Formabilities   |              | Panel performance |               |  |
|     |       |                       |           |             |             |                            |                            |              |            | Plane<br>strain | ΔWca<br>(μm) | Dent load<br>(N)  | baking<br>(N) |  |
| 22  | 11    | CAL                   | 184       | 13          | 0.242       | 0.246                      | 30.3                       | 2.16         | None       | 0               | 90           | 165               |               |  |
| 23  |       | CGL                   | 185       | 14          | 0.235       | 0.230                      | 29.7                       | 2.14         | None       | 0               | 91           | 168               |               |  |
| 24  | 12    | CAL                   | 238       | 11          | 0.259       | 0.261                      | 31.4                       | 2.17         | None       | 0               | 88           | 186               |               |  |
| 25  |       | CGL                   | 237       | 13          | 0.253       | 0.244                      | 31.3                       | 2.15         | None       | 0               | 90           | 186               |               |  |
| 26  | 13    | CAL                   | 180       | 0           | 0.242       | 0.253                      | 31.5                       | 2.18         | None       | 0               | 60           | 145               |               |  |
| 27  | 14    | CAL                   | 170       | 0           | 0.248       | 0.261                      | 31.8                       | 2.19         | None       | 0.2             | 54           | 126               |               |  |
| 28  | 15    | CAL                   | 205       | 23          | 0.265       | 0.263                      | 30.9                       | 2.14         | None       | 0.1             | 96           | 179               |               |  |
| 29  |       | CGL                   | 205       | 25          | 0.247       | 0.245                      | 30.6                       | 2.13         | None       | 0               | 98           | 175               |               |  |
| 30  | 16    | CAL                   | 235       | 37          | 0.243       | 0.198                      | 29.4                       | 2.09         | Permissive | 0.2             | 101          | 177               |               |  |
| 31  |       | CGL                   | 238       | 38          | 0.237       | 0.197                      | 29.2                       | 2.05         | Permissive | 0.2             | 104          | 177               |               |  |
| 32  | 17    | CAL                   | 250       | 40          | 0.195       | 0.251                      | 28.8                       | 2.04         | Inferior   | 0.4             | 107          | 179               |               |  |
| 33  | 18    | CAL                   | 233       | 31          | 0.197       | 0.251                      | 29.8                       | 2.11         | None       | 0               | 98           | 183               |               |  |
| 34  |       | CGL                   | 231       | 30          | 0.195       | 0.253                      | 29.9                       | 2.1          | None       | 0               | 96           | 180               |               |  |
| 35  | 19    | CAL                   | 235       | 27          | 0.195       | 0.253                      | 30.1                       | 2.13         | None       | 0               | 105          | 176               |               |  |
| 36  |       | CGL                   | 235       | 25          | 0.196       | 0.252                      | 30                         | 2.11         | None       | 0               | 103          | 172               |               |  |
| 37  | 20    | CAL                   | 249       | 43          | 0.183       | 0.190                      | 29.5                       | 2.07         | Inferior   | 0.4             | 109          | 185               |               |  |
| 38  |       | CGL                   | 253       | 41          | 0.180       | 0.192                      | 29.3                       | 2.07         | Inferior   | 0.4             | 110          | 183               |               |  |
| 39  | 21    | CAL                   | 261       | 39          | 0.181       | 0.189                      | 29.1                       | 2.05         | Inferior   | 0.2             | 113          | 185               |               |  |

TABLE 4-continued

| No. | Steel No. | Mechanical properties         |          |               |                         |                         |           |      |              | Dent load |               |            |
|-----|-----------|-------------------------------|----------|---------------|-------------------------|-------------------------|-----------|------|--------------|-----------|---------------|------------|
|     |           | Work-hardening exponent:<br>n |          | Formabilities |                         | Panel performance       |           |      | after        |           |               |            |
|     |           | Annealing                     | YP (MPa) | BH (MPa)      | Strain rate :3 x 10-3/s | Strain rate :3 x 10-1/s | LDH0 (mm) | LDR  | Plane strain | ΔWca (μm) | Dent load (N) | baking (N) |
| 40  | 22        | CAL                           | 205      | 30            | 0.274                   | 0.271                   | 31.6      | 2.16 | None         | 0         | 91            | 172        |
| 41  | 23        | CAL                           | 213      | 25            | 0.269                   | 0.270                   | 31.5      | 2.16 | None         | 0         | 92            | 173        |

TABLE 5

| No. | Steel No. | Mechanical properties         |          |               |                         |                         |           |      |              | Dent load |               |            |
|-----|-----------|-------------------------------|----------|---------------|-------------------------|-------------------------|-----------|------|--------------|-----------|---------------|------------|
|     |           | Work-hardening exponent:<br>n |          | Formabilities |                         | Panel performance       |           |      | after        |           |               |            |
|     |           | Annealing                     | YP (MPa) | BH (MPa)      | Strain rate :3 x 10-3/s | Strain rate :3 x 10-1/s | LDH0 (mm) | LDR  | Plane strain | ΔWca (μm) | Dent load (N) | baking (N) |
| 42  | 24        | CAL                           | 221      | 24            | 0.265                   | 0.261                   | 31.2      | 2.15 | None         | 0         | 95            | 175        |
| 43  |           | CGL                           | 222      | 26            | 0.251                   | 0.253                   | 30.8      | 2.14 | None         | 0         | 94            | 175        |
| 44  | 25        | CAL                           | 201      | 0             | 0.248                   | 0.237                   | 30.5      | 2.17 | None         | 0         | 60            | 147        |
| 45  | 26        | CAL                           | 215      | 0             | 0.229                   | 0.227                   | 30.2      | 2.14 | None         | 0         | 62            | 149        |
| 46  | 27        | CAL                           | 221      | 31            | 0.267                   | 0.265                   | 30.4      | 2.15 | None         | 0.1       | 92            | 173        |
| 47  | 28        | CAL                           | 203      | 0             | 0.193                   | 0.200                   | 30.1      | 2.14 | None         | 0         | 79            | 148        |
| 48  | 29        | CAL                           | 195      | 0             | 0.245                   | 0.243                   | 31.3      | 2.16 | None         | 0         | 75            | 147        |
| 49  |           | CGL                           | 194      | 0             | 0.252                   | 0.239                   | 31.2      | 2.15 | None         | 0         | 74            | 146        |
| 50  | 30        | CAL                           | 205      | 15            | 0.262                   | 0.260                   | 30.9      | 2.15 | None         | 0         | 90            | 173        |
| 51  |           | CGL                           | 207      | 15            | 0.258                   | 0.255                   | 30.7      | 2.13 | None         | 0         | 92            | 174        |
| 52  | 31        | CAL                           | 237      | 27            | 0.197                   | 0.256                   | 30.2      | 2.14 | None         | 0         | 98            | 183        |
| 53  |           | CGL                           | 236      | 28            | 0.198                   | 0.254                   | 30.0      | 2.13 | None         | 0         | 94            | 180        |
| 54  | 32        | CAL                           | 213      | 17            | 0.253                   | 0.256                   | 30.8      | 2.11 | None         | 0         | 93            | 175        |
| 55  | 33        | CAL                           | 203      | 0             | 0.215                   | 0.180                   | 30.4      | 2.13 | None         | 0         | 75            | 149        |
| 56  | 34        | CAL                           | 235      | 24            | 0.256                   | 0.253                   | 29.8      | 2.11 | None         | 0         | 104           | 182        |
| 57  |           | CGL                           | 234      | 26            | 0.251                   | 0.256                   | 29.7      | 2.1  | None         | 0         | 108           | 180        |
| 58  | 35        | CAL                           | 246      | 40            | 0.212                   | 0.192                   | 27.9      | 2.16 | Permissive   | 0.2       | 106           | 187        |
| 59  |           | CGL                           | 252      | 42            | 0.205                   | 0.194                   | 27.8      | 2.13 | Inferior     | 0.2       | 110           | 189        |

TABLE 6

| No. | Steel No. | Mechanical properties |                       |           |          |                               |                         |               |      | Dent load         |           |               |            |
|-----|-----------|-----------------------|-----------------------|-----------|----------|-------------------------------|-------------------------|---------------|------|-------------------|-----------|---------------|------------|
|     |           | Coiling               |                       | Annealing |          | Work-hardening exponent:<br>n |                         | Formabilities |      | Panel performance |           |               |            |
|     |           | Coiling temp. (°C.)   | Annealing temp. (°C.) | YP (MPa)  | BH (MPa) | Strain rate :3 x 10-3/s       | Strain rate :3 x 10-1/s | LDH0 (mm)     | LDR  | Plane strain      | ΔWca (μm) | Dent load (N) | baking (N) |
| 60  | 5         | 680                   | 840                   | 216       | 21       | 0.272                         | 0.27                    | 31.1          | 2.16 | None              | 0         | 90            | 173        |
| 61  | 5         | 640                   | 840                   | 217       | 22       | 0.275                         | 0.273                   | 30.9          | 2.13 | None              | 0         | 92            | 178        |
| 62  | 5         | 640                   | 880                   | 209       | 24       | 0.273                         | 0.272                   | 31.2          | 2.15 | None              | 0         | 89            | 170        |
| 63  | 5         | 720                   | 880                   | 178       | 32       | 0.263                         | 0.266                   | 29.5          | 2.17 | None              | 0.4       | 80            | 161        |
| 64  | 5         | 640                   | 920                   | 250       | 42       | 0.243                         | 0.243                   | 28.7          | 2.01 | Inferior          | 0         | 102           | 183        |
| 65  | 6         | 640                   | 840                   | 203       | 0        | 0.237                         | 0.197                   | 31.1          | 2.16 | None              | 0         | 58            | 145        |
| 66  | 6         | 640                   | 860                   | 201       | 5        | 0.236                         | 0.195                   | 31.4          | 2.18 | None              | 0         | 64            | 148        |
| 67  | 6         | 640                   | 880                   | 198       | 18       | 0.244                         | 0.188                   | 31.7          | 2.2  | None              | 0.3       | 72            | 146        |
| 68  | 6         | 700                   | 880                   | 175       | 17       | 0.240                         | 0.196                   | 30.8          | 2.22 | None              | 0.8       | 68            | 144        |
| 69  | 12        | 640                   | 860                   | 238       | 11       | 0.259                         | 0.261                   | 31.4          | 2.17 | None              | 0         | 88            | 186        |
| 70  | 12        | 640                   | 880                   | 231       | 20       | 0.257                         | 0.258                   | 31.6          | 2.2  | None              | 0         | 86            | 181        |
| 71  | 12        | 640                   | 920                   | 275       | 32       | 0.198                         | 0.232                   | 28.9          | 1.98 | Inferior          | 0.2       | 115           | 191        |
| 72  | 25        | 640                   | 860                   | 201       | 0        | 0.248                         | 0.237                   | 30.5          | 2.17 | None              | 0         | 60            | 147        |

TABLE 7

| No. | Steel No. | Mechanical properties |                       |           |          |                               |                         |               |      | Dent load         |           |               |            |
|-----|-----------|-----------------------|-----------------------|-----------|----------|-------------------------------|-------------------------|---------------|------|-------------------|-----------|---------------|------------|
|     |           | Coiling               |                       | Annealing |          | Work-hardening exponent:<br>n |                         | Formabilities |      | Panel performance |           |               |            |
|     |           | Coiling temp. (°C.)   | Annealing temp. (°C.) | YP (MPa)  | BH (MPa) | Strain rate :3 x 10-3/s       | Strain rate :3 x 10-1/s | LDH0 (mm)     | LDR  | Plane strain      | ΔWca (μm) | Dent load (N) | baking (N) |
| 73  | 25        | 640                   | 880                   | 197       | 15       | 0.246                         | 0.233                   | 30.8          | 2.2  | None              | 0.3       | 68            | 148        |
| 74  | 25        | 640                   | 900                   | 181       | 28       | 0.249                         | 0.236                   | 29.8          | 2.21 | Permissive        | 0.6       | 70            | 149        |

TABLE 7-continued

| No. | Steel No. | Mechanical properties |                       |                          |          |                         |                         |           |                   |              |           | Dent load after baking (N) |     |
|-----|-----------|-----------------------|-----------------------|--------------------------|----------|-------------------------|-------------------------|-----------|-------------------|--------------|-----------|----------------------------|-----|
|     |           | Coiling temp. (°C.)   | Annealing temp. (°C.) | Work-hardening exponent: |          |                         | Formabilities           |           | Panel performance |              |           |                            |     |
|     |           |                       |                       | YP (MPa)                 | BH (MPa) | Strain rate :3 x 10-3/s | Strain rate :3 x 10-1/s | LDH0 (mm) | LDR               | Plane strain | ΔWca (μm) | Dent load (N)              |     |
| 75  | 25        | 680                   | 860                   | 198                      | 0        | 0.247                   | 0.219                   | 30.9      | 2.18              | Permissive   | 0         | 59                         | 145 |
| 76  | 29        | 640                   | 860                   | 195                      | 0        | 0.245                   | 0.243                   | 31.3      | 2.16              | None         | 0         | 75                         | 147 |
| 77  | 29        | 640                   | 880                   | 188                      | 13       | 0.249                   | 0.245                   | 31.1      | 2.18              | None         | 0.3       | 74                         | 149 |
| 78  | 29        | 640                   | 900                   | 183                      | 15       | 0.243                   | 0.24                    | 30.4      | 2.05              | None         | 0.7       | 71                         | 142 |
| 79  | 29        | 680                   | 860                   | 193                      | 0        | 0.244                   | 0.237                   | 31.6      | 2.19              | None         | 0         | 73                         | 145 |
| 80  | 30        | 640                   | 860                   | 205                      | 15       | 0.262                   | 0.26                    | 30.9      | 2.15              | None         | 0         | 90                         | 173 |
| 81  | 30        | 680                   | 880                   | 202                      | 20       | 0.268                   | 0.257                   | 31.2      | 2.18              | None         | 0         | 91                         | 176 |
| 82  | 30        | 680                   | 860                   | 201                      | 13       | 0.26                    | 0.252                   | 30.7      | 2.17              | None         | 0         | 90                         | 171 |
| 83  | 30        | 700                   | 880                   | 172                      | 22       | 0.271                   | 0.254                   | 30.4      | 2.21              | None         | 0.4       | 77                         | 148 |
| 84  | 31        | 640                   | 840                   | 237                      | 27       | 0.197                   | 0.256                   | 30.2      | 2.14              | None         | 0         | 98                         | 183 |
| 85  | 31        | 680                   | 860                   | 230                      | 28       | 0.199                   | 0.253                   | 30.5      | 2.17              | None         | 0         | 94                         | 180 |
| 86  | 31        | 680                   | 880                   | 220                      | 31       | 0.195                   | 0.251                   | 30.1      | 2.02              | None         | 0         | 99                         | 182 |
| 87  | 31        | 700                   | 900                   | 246                      | 38       | 0.188                   | 0.238                   | 28.6      | 2.00              | Permissive   | 0.2       | 102                        | 187 |

What is claimed is:

1. A cold-rolled steel sheet for excellent panel appearance and dent resistance after panel-forming, comprising a steel composition containing 0.0010 to 0.01 wt % of C, 0 to 0.2 wt % of Si, 0.1 to 1.5 wt % of Mn, 0 to 0.05 wt % of P, 0 to 0.02 wt % of S, 0.03 to 0.10 wt % of sol. Al, and 0 to 0.0040 wt % of N, and further containing one or both of 0.005 to 0.08 wt % of Nb and 0.01 to 0.07 wt % of Ti in the ranges given by the following formulae (1) and (2):

$$\{(12/93)Nb+(12/48)Ti^*\} \geq 0.0005 \quad (1)$$

$$0 \leq C - \{(12/93)Nb+(12/48)Ti^*\} \leq 0.0015 \quad (2)$$

wherein  $Ti^* = Ti - \{(48/32)S+(48/14)N\}$

said cold-rolled steel sheet having a bake hardenability BH of 10 to 35 MPa obtained by a 2% tensile prestrain and 170° C.×20 min heat treatment;

said bake hardenability BH (MPa) and a yield strength YP (MPa) of said steel sheet satisfying the following formulae (3a) and (4a)

$$BH \geq \exp(-0.115 \cdot YP + 23.0) \quad (3a)$$

$$0.67 \cdot BH + 160 \leq YP \leq -0.8 \cdot BH + 280 \quad (4a)$$

2. A cold-rolled steel sheet for excellent panel appearance and dent resistance after panel-forming, comprising a steel composition containing 0.0010 to 0.01 wt % of C, 0 to 0.2 wt % of Si, 0.1 to 1.5 wt % of Mn, 0 to 0.05 wt % of P, 0 to 0.02 wt % of S, 0.03 to 0.10 wt % of sol. Al, and 0 to 0.0040 wt % of N, and further containing one or both of 0.005 to 0.08 wt % of Nb and 0.01 to 0.07 wt % of Ti in the ranges given by the following formulae (1) and (2):

$$\{(12/93)Nb+(12/48)Ti^*\} \geq 0.0005 \quad (1)$$

$$0 \leq C - \{(12/93)Nb+(12/48)Ti^*\} \leq 0.0015 \quad (2)$$

wherein  $Ti^* = Ti - \{(48/32)S+(48/14)N\}$

said cold-rolled steel sheet having a bake hardenability BH of 10 to 30 MPa obtained by 2% tensile prestrain and 170° C.×20 min heat treatment;

said bake hardenability BH (MPa) and a yield strength YP (MPa) of said steel sheet satisfying the following formulae (3b) and (4b)

$$BH \geq \exp(-0.115 \cdot YP + 25.3) \quad (3b)$$

$$0.67 \cdot BH + 177 \leq YP \leq -0.8 \cdot BH + 260 \quad (4b)$$

3. A cold-rolled steel sheet for excellent panel appearance and dent resistance after panel-forming, comprising a steel composition containing 0.0010 to 0.0025 wt % of C, 0 to 0.2 wt % of Si, 0.1 to 1.5 wt % of Mn, 0 to 0.05 wt % of P, 0 to 0.02 wt % of S, 0.03 to 0.10 wt % of sol. Al, and 0 to 0.0040 wt % of N, and further containing one or both of 0.005 to 0.020 wt % of Nb and 0.01 to 0.05 wt % of Ti in the ranges given by the following formulae (1) and (2):

$$\{(12/93)Nb+(12/48)Ti^*\} \geq 0.0005 \quad (1)$$

$$0 \leq C - \{(12/93)Nb+(12/48)Ti^*\} \leq 0.0015 \quad (2)$$

wherein  $Ti^* = Ti - \{(48/32)S+(48/14)N\}$

said cold-rolled steel sheet having a bake hardenability BH of 10 to 35 MPa obtained by a 2% tensile prestrain and 170° C.×20 min heat treatment;

said bake hardenability BH (MPa) and a yield strength YP (MPa) of said steel sheet satisfying the following formulae (3a) and (4a)

$$BH \geq \exp(-0.115 \cdot YP + 23.0) \quad (3a)$$

$$0.67 \cdot BH + 160 \leq YP \leq -0.8 \cdot BH + 280 \quad (4a)$$

4. A cold-rolled steel sheet for excellent panel appearance and dent resistance after panel-forming, comprising a steel composition containing 0.0010 to 0.0025 wt % of C, 0 to 0.2 wt % of Si, 0.1 to 1.5 wt % of Mn, 0 to 0.05 wt % of P, 0 to 0.02 wt % of S, 0.03 to 0.10 wt % of sol. Al, and 0 to 0.0040 wt % of N, and further containing one or both of 0.005 to 0.020 wt % of Nb and 0.01 to 0.05 wt % of Ti in the ranges given by the following formulae (1) and (2):

$$\{(12/93)Nb+(12/48)Ti^*\} \geq 0.0005 \quad (1)$$

$$0 \leq C - \{(12/93)Nb+(12/48)Ti^*\} \leq 0.0015 \quad (2)$$

wherein  $Ti^* = Ti - \{(48/32)S+(48/14)N\}$

said cold-rolled steel sheet having a bake hardenability BH of 10 to 30 MPa obtained by 2% tensile prestrain and 170° C.×20 min heat treatment;

said bake hardenability BH (MPa) and a yield strength YP (MPa) of said steel sheet satisfying the following formulae (3b) and (4b)

$$BH \geq \exp(-0.115 \cdot YP + 25.3) \quad (3b)$$

$$0.67 \cdot BH + 177 \leq YP \leq -0.8 \cdot BH + 260 \quad (4b)$$

**19**

0.67-BH+177≤YP≤-0.8-BH+260

(4b).

5. The cold-rolled steel sheet of claim 1, wherein said steel composition contains 0.0002 to 0.0015 wt % of B.

6. A cold-rolled steel sheet of claim 1,

5 wherein said cold-rolled steel sheet is coated with a zinc or zinc alloy layer.

7. The cold-rolled steel sheet of claim 1, wherein the steel sheet has a composition selected from the group consisting of

- (a) 0.0019 wt % C, 0.02 wt % Si, 0.56 wt % Mn, 0.35 wt % P, 0.011 wt % S, 0.044 wt % sol.Al, 0.0021 wt % N, 0.006 wt % Nb, with the remainder being Fe;
- (b) 0.0023 wt % C, 0.01 wt % Si, 0.48 wt % Mn, 0.028 wt % P, 0.009 wt % S, 0.0045 wt % sol.Al, 0.0018 wt % N, 0.011 wt % Nb, with the remainder being Fe;
- (c) 0.0018 wt % C, 0.02 wt % Si, 0.92 wt % Mn, 0.032 wt % P, 0.007 wt % S, 0.054 wt % sol.Al, 0.0016 wt % N, 0.009 wt % Nb, with the remainder being Fe;
- (d) 0.0022 wt % C, 0.01 wt % Si, 0.25 wt % Mn, 0.029 wt % P, 0.012 wt % S, 0.043 wt % sol.Al, 0.0025 wt % N, 0.009 wt % Nb, with the remainder being Fe;
- (e) 0.0019 wt % C, 0.01 wt % Si, 1.25 wt % Mn, 0.014 wt % P, 0.009 wt % S, 0.041 wt % sol.Al, 0.0024 wt % N, 0.015 wt % Nb, with the remainder being Fe;
- (f) 0.005 wt % C, 0.02 wt % Si, 0.35 wt % Mn, 0.042 wt % P, 0.01 wt % S, 0.051 wt % sol.Al, 0.0022 wt % N, 0.029 wt % Nb, with the remainder being Fe;
- (g) 0.007 wt % C, 0.01 wt % Si, 0.66 wt % Mn, 0.025 wt % P, 0.011 wt % S, 0.041 wt % sol.Al, 0.0019 wt % N, 0.046 wt % Nb, with the remainder being Fe;
- (h) 0.0021 wt % C, 0.01 wt % Si, 0.52 wt % Mn, 0.039 wt % P, 0.009 wt % S, 0.048 wt % sol.Al, 0.0018 wt % N, 0.023 wt % Ti, with the remainder being Fe;
- (i) 0.0021 wt % C, 0.02 wt % Si, 0.53 wt % Mn, 0.039 wt % P, 0.018 wt % S, 0.052 wt % sol.Al, 0.0039 wt % N, 0.045 wt % Ti, with the remainder being Fe;

**20**

(j) 0.0022 wt % C, 0.01 wt % Si, 0.53 wt % Mn, 0.039 wt % P, 0.018 wt % S, 0.052 wt % sol.Al, 0.0039 wt % N, 0.045 wt % Ti, with the balance being Fe;

(k) 0.0023 wt % C, 0.01 wt % Si, 0.48 wt % Mn, 0.025 wt % P, 0.012 wt % S, 0.044 wt % sol.Al, 0.0022 wt % N, 0.055 wt % Ti, with the balance being Fe;

(l) 0.0019 wt % C, 0.01 wt % Si, 0.53 wt % Mn, 0.024 wt % P, 0.009 wt % S, 0.066 wt % sol.Al, 0.0017 wt % N, 0.014 wt % Nb, 0.024 wt % Ti, with the remainder being Fe; and

(m) 0.0085 wt % C, 0.01 wt % Si, 0.37 wt % Mn, 0.03 wt % P, 0.01 wt % S, 0.051 wt % sol.Al, 0.0018 wt % N, 0.04 wt % Nb, 0.03 wt % Ti, with the remainder being Fe.

8. The cold-rolled steel sheet of claim 1, wherein the steel composition includes 0.005 to 0.08 wt % Nb.

9. The cold-rolled steel sheet of claim 1, wherein the steel composition includes 0.01 to 0.07 wt % Ti.

10. The cold-rolled steel sheet of claim 1, wherein the steel composition includes 0.005 to 0.08 wt % Nb and 0.01 to 0.07 wt % Ti.

11. The cold-rolled steel sheet of claim 5, wherein the steel sheet has a composition selected from the group consisting of

(a) 0.0021 wt % C, 0.02 wt % Si, 0.43 wt % Mn, 0.034 wt % P, 0.012 wt % S, 0.042 wt % sol.Al, 0.0021 wt % N, 0.001 wt % Nb, 0.0008 wt % B, with the remainder being Fe;

(b) 0.0024 wt % C, 0.01 wt % Si, 0.43 wt % Mn, 0.032 wt % P, 0.011 wt % S, 0.062 wt % sol.Al, 0.0026 wt % N, 0.033 wt % Ti, 0.0009 wt % B, with the remainder being Fe; and

(c) 0.0021 wt % C, 0.02 wt % Si, 0.38 wt % Mn, 0.023 wt % P, 0.008 wt % S, 0.052 wt % sol.Al, 0.0019 wt % N, 0.009 wt % Nb, 0.018 wt % Ti, 0.0005 wt % B, with the remainder being Fe.

\* \* \* \* \*